# EUROPEAN PATENT APPLICATION

(11) **EP 4 748 992 A1**
(43) Date of publication of application: **27.05.2026**
(21) Application number: 24842859.1
(22) Date of filing: 12.06.2024
(51) Int. Cl.: D04B 21/12, A41D 31/14, D01F 8/14, D02G 1/02, D04B 21/16

(54) **MESH KNITTED FABRIC AND FIBER PRODUCT**

(30) Priority: 20.07.2023 JP 2023117969
(71) Applicant: TEIJIN FRONTIER CO., LTD., Osaka-shi, Osaka 530-0005 (JP)
(72) Inventor: UMEDA Ryota, Osaka-shi, Osaka 530-0005 (JP); OGATA Nobuaki, Osaka-shi, Osaka 530-0005 (JP)
(74) Representative: Carpmaels & Ransford LLP
(86) International application number: PCT/JP2024/021267
(87) International publication number: WO 2025/018063

(57) **Abstract**

A task is to provide a mesh knitted fabric which is reversibly increased in the area of a mesh part when being wetted, enabling the self-regulating function of the fabric to be visually recognized, and a fiber product, and a means for solving the problem is a mesh knitted fabric having a mesh part, wherein the mesh knitted fabric comprises a yarn composed of a conjugate fiber having a polyester component and a polyamide component bonded in a side-by-side form, wherein the area of the mesh part of the mesh knitted fabric upon being wetted is increased.

## Description

### Technical Field

The present invention relates to a mesh knitted fabric which is reversibly increased in the area of a mesh part when being wetted, enabling the self-regulating function of the fabric to be visually recognized, and a fiber product.

### Background Art

Conventionally, as a self-regulating fabric which is reversibly improved in air permeability, for example, when being wetted, a fabric using a yarn composed of a conjugate fiber having a polyester component and a polyamide component bonded in a side-by-side form has been proposed (PTLs 1 and 2) .

Such a conventional fabric has a self-regulating function, but it has been difficult to visually recognize the change of the self-regulating function of the fabric, for example, a change of the size of a mesh part (void).

### Citation List

### Patent Literature

PTL 1: JP2006-97147A
PTL 2: WO2017/038239 pamphlet

### Summary of Invention

### Technical Problem

In view of the above, the present invention has been made, and an object of the present invention is to provide a mesh knitted fabric which is reversibly increased in the area of a mesh part when being wetted, enabling the self-regulating function of the fabric to be visually recognized, and a fiber product.

### Solution to Problem

The present inventor has conducted extensive and intensive studies with a view toward achieving the above-mentioned task. As a result, the inventor has focused on the fact that, with respect to a mesh knitted fabric having a ground structure part and a connecting part for connecting a ground structure part and another one, when a yarn which stretches in the long direction upon being wetted is used in the connecting part, the area of a mesh part (void) of the fabric upon being wetted is increased, and further extensive and intensive studies have been made, so that the present invention has been completed. Thus, the following invention is provided.

1. A mesh knitted fabric having a mesh part, wherein the mesh knitted fabric comprises a yarn composed of a conjugate fiber having a polyester component and a polyamide component bonded in a side-by-side form, wherein the area of the mesh of the mesh knitted fabric upon being wetted is increased, as compared to the area of the mesh before wetted.
2. The mesh knitted fabric according to item 1 above, wherein the size of the one mesh part is in the range of from 2 to 12 courses.
3. The mesh knitted fabric according to item 1 or 2 above, which further comprises a composite yarn containing a false-twisted crimped yarn having a torque in the S direction and a false-twisted crimped yarn having a torque in the Z direction.
4. The mesh knitted fabric according to any one of items 1 to 3 above, which has a warp-knitted fabric structure.
5. The mesh knitted fabric according to any one of items 1 to 4 above, which has a knitted fabric density wherein the number of courses is 20 to 100/2.54 cm and the number of wales is 20 to 80/2.54 cm.
6. The mesh knitted fabric according to any one of items 1 to 5 above, which contains a water absorption imparting agent.
7. The mesh knitted fabric according to any one of items 1 to 6 above, which has a fiber areal weight in the range of from 50 to 250 g/m².
8. The mesh knitted fabric according to items 1 to 7 above, which has an air permeability change ratio of 5% or more when being wetted.
9. The mesh knitted fabric according to any one of claims 1 to 8 above, which has a dimensional change ratio of 10% or less in the lengthwise direction and a dimensional change ratio of 15% or less in the widthwise direction when being wetted.
10. A fiber product which is obtained using the mesh knitted fabric according to any one of items 1 to 9 above, wherein the fiber product is selected from the group consisting of clothes, a backing fabric, a core fabric, socks, a stomach band, a hat, gloves, nightclothes, a casing material for futon (thick bedquilt), a cover for futon, and a car seat skin material.

### Advantageous Effects of Invention

In the present invention, there are obtained a mesh knitted fabric which is reversibly increased in the area of a mesh part when being wetted, enabling the self-regulating function of the fabric to be visually recognized, and a fiber product.

### Brief Description of Drawings

[FIG. 1] FIG. 1 is a knitted structure pattern used in Example 1.
[FIG. 2] FIG. 2 is a knitted structure pattern used in Comparative Example 1.
[FIG. 3] FIG. 3 is a diagram of the knitted structure used in Example 1.

### Description of Embodiments

Hereinbelow, an embodiment of the present invention will be described in detail. First, the invention is directed to a mesh knitted fabric (hereinafter, referred to also as "cloth") having a mesh part (void), wherein the mesh knitted fabric comprises a yarn composed of a conjugate fiber having a polyester component and a polyamide component bonded in a side-by-side form, wherein the area of the mesh part of the mesh knitted fabric upon being wetted is increased, as compared to the area of the mesh part before wetted.

As diagrammatically shown in FIG. 3, the mesh knitted fabric of the invention has a mesh part, a ground structure part, and a connecting part. The connecting parts are positioned so as to sandwich a mesh part therebetween, and connect a ground structure part and another ground structure part. The yarn composed of the conjugate fiber is used in the connecting part, and therefore, when the mesh knitted fabric is wetted, the yarn composed of the conjugate fiber stretches in the widthwise direction (in the direction indicated by an arrow), and accordingly, the mesh part also expands in the widthwise direction, and expansion of the mesh part can be visually observed.

The mesh part is formed by, for example, conducting raveling for a reed when knitting the warp-knitted fabric, forming a part in which a wale and another wale are not connected through a loop. Specifically, the yarn composed of the conjugate fiber is used in the connecting part, and the yarn composed of the conjugate fiber is arranged in end portions of the mesh part, so that a mesh structure is obtained in which the mesh part is surrounded by the yarn composed of the conjugate fiber.

The size of the one mesh part (void) is preferably in the range of from 2 to 12 courses (more preferably 2 to 8 courses) and one or more wales (more preferably 1 to 4 wales).

With respect to the polyester component of the conjugate fiber, in view of the adhesion to the polyamide component which is the other component of the conjugate fiber, preferred examples of the polyester include modified polyesters obtained by copolymerizing a compound, which has an alkali metal or alkaline earth metal salt or phosphonium salt of sulfonic acid, or the like, and which has at least one functional group having ester formability, with polyethylene terephthalate, polypropylene terephthalate, polybutylene terephthalate, or the like. Of these, in view of the general-purpose properties and polymer cost, especially preferred is modified polyethylene terephthalate having the above-mentioned compound copolymerized therewith. As examples of the copolymerizable components used in the modified polyester, there can be mentioned sodium 5-sulfoisophthalate and an ester derivative thereof, 5-phosphonium isophthalate and an ester derivative thereof, and sodium p-hydroxybenzenesulfonate. Of these, sodium 5-sulfoisophthalate is preferred. The amount of the copolymerized compound is preferably in the range of from 2.0 to 4.5 mol%. When the amount of the copolymerized compound is smaller than 2.0 mol%, excellent crimping performance is obtained, but there is a danger that a removal is caused in the interface between the polyamide component and polyester component bonded together. On the other hand, when the amount of the copolymerized compound is larger than 4.5 mol%, crystallization of the polyester component is unlikely to proceed during a drawing heat treatment, and therefore the temperature for the drawing heat treatment needs to be increased, leading to a disadvantage in that yarn breaking frequently occurs.

On the other hand, with respect to the polyamide component, there is no particular limitation as long as the component has an amide linkage in the main chain thereof, and examples of such components include nylon 4, nylon 6, nylon 66, nylon 46, and nylon 12. Of these, in view of the general-purpose properties, polymer cost, and stability of yarn production, nylon 6 and nylon 66 are preferred.

The polyester component and polyamide component may contain a known additive, such as a pigment, a matting agent, a stainproofing agent, a fluorescent brightener, a flame retardant, a stabilizer, an antistatic agent, a light stabilizer, or an ultraviolet light absorber.

The conjugate fiber having a polyester component and a polyamide component bonded in a side-by-side form can have an arbitrary cross-sectional shape and conjugate form. The conjugate fiber may have a form of eccentric core/sheath. Further, the conjugate fiber may have a triangular cross-sectional shape or a rectangular cross-sectional shape, or may have a hollow portion in the cross-section thereof. Especially, preferred is a conjugate fiber such that the single fiber cross-sectional shape is circular and the conjugate fiber has a side-by-side form. The ratio of the polyester and polyamide components in the conjugate fiber can be arbitrarily selected, but is preferably in the range of from 30:70 to 70:30 (more preferably 40:60 to 60:40), in terms of a weight ratio of the two components.

In the yarn composed of the conjugate fiber, with respect to the single fiber fineness and the number of filaments (the number of single fibers), there is no particular limitation, but the single fiber fineness is preferably in the range of from 0.1 to 10 dtex (more preferably 0.8 to 3.5 dtex), and the number of filaments is preferably in the range of from 10 to 200 (more preferably 20 to 100). Especially, preferred is a multifilament (continuous fiber) having a single fiber fineness of 0.8 to 3.5 dtex and a total fineness of 20 to 110 dtex.

A conjugate fiber having different polymers bonded in a side-by-side form generally has a latent crimping performance and, as mentioned below, exhibits latent crimping performance when subjected to heat treatment in dyeing or the like. With respect to the crimped structure of the conjugate fiber, preferred is a crimped structure in which the polyamide component is positioned inside of the crimps and the polyester component is positioned outside of the crimps. In the conjugate fiber having such a crimped structure, when being wetted, the polyamide component positioned inside swells and stretches, and the polyester component positioned outside causes almost no change in the length, so that the crimp degree is reduced (the apparent length of the conjugate fiber is increased). On the other hand, when being dried, the polyamide component positioned inside shrinks, and the polyester component positioned outside causes almost no change in the length, so that the crimp degree is increased (the apparent length of the conjugate fiber is reduced).

In view of obtaining a mesh knitted fabric which is easily reduced in crimps when being wetted to be efficiently improved in air permeability, the yarn composed of the conjugate fiber is preferably a non-twisted yarn or a soft twisted yarn which has been twisted at 300 T/m or less. Particularly, the yarn composed of the conjugate fiber is preferably a non-twisted yarn. When the yarn composed of the conjugate fiber is strongly twisted like a strong twisted yarn, there is a disadvantage in that the resultant knitted fabric is unlikely to be reduced in crimps upon being wetted. The yarn may have been subjected to air interlacing and/or general false-twist crimping so that the number of interlaces becomes about 20 to 100/m (more preferably 20 to 60/m).

The yarn composed of the conjugate fiber can be produced by the method described in WO2017/038239 pamphlet.

In the mesh knitted fabric of the invention, with respect to the yarn used in the ground structure part, there is no particular limitation, and the yarn may be a non-crimped yarn or may be a false-twisted crimped yarn. For example, the yarn may be a composite yarn (crimped fiber) containing a false-twisted crimped yarn having a torque in the S direction and a false-twisted crimped yarn having a torque in the Z direction. Such a composite yarn is described in WO2017/038239 pamphlet, and, when the ground structure part is formed from the composite yarn, an advantage is obtained such that the resultant knitted fabric has a flat surface and thus has an improved snagging resistance.

The yarn used in the ground structure part preferably has a single fiber fineness of 2.3 dtex or less (preferably 0.00002 to 2.0 dtex, especially preferably 0.1 to 1.0 dtex). The smaller the single fiber fineness of the yarn, the more excellent the yarn is, and the yarn may be a yarn having a single fiber diameter of 1,000 nm or less, which is called a nanofiber. When the single fiber fineness of the yarn is larger than 2.3 dtex, there is a danger that the water absorption properties of the mesh knitted fabric become poor, so that the air permeability change ratio is lowered upon being wetted. It is preferred that the single fiber fineness of the yarn used in the ground structure part is smaller than the single fiber fineness of the conjugate fiber. Further, the yarn used in the ground structure part preferably has a total fineness in the range of from 33 to 220 dtex. Furthermore, with respect to the yarn used in the ground structure part, the number of filaments is preferably in the range of from 30 to 300 (more preferably 40 to 200).

Further, with respect to the yarn used in the ground structure part, the single fiber cross-sectional shape may be a shape of a general circular cross-section, but may be a shape of an irregular-shaped cross-section other than the circular cross-section. Examples of shapes of such an irregular-shaped cross-section include triangle, rectangle, a cruciform shape, a flattened shape, a flattened shape having a shoulder, an H-shape, and a W-shape. With respect to the flattened cross-sectional shape, a flatness of the cross-section represented by B/C1, which is the ratio of the length B of the cross-section in the longitudinal central line direction to the maximum width C1 in the direction perpendicular to the longitudinal central line direction, is preferably in the range of from 2 to 6 (more preferably 3.1 to 5.0) in view of the softness of the cloth. Further, the ratio of the maximum width C1 of the cross-section to the minimum width C2, i.e., the C1/C2 ratio is preferably in the range of from 1.05 to 4.00 (more preferably 1.1 to 1.5) in view of the water absorption properties of the cloth.

With respect to the fiber constituting the yarn used in the ground structure part, there is no particular limitation, and there can be used a polyester fiber, an acrylic fiber, a nylon fiber, a rayon fiber, an acetate fiber, a natural fiber, such as cotton, wool, or silk, or a conjugate fiber thereof. Particularly, a polyester fiber composed of the above-mentioned polyester is preferred.

The mesh knitted fabric of the invention may be a circular knitted fabric, but is preferably a warp-knitted fabric. Preferred examples of structures of the ground structure part of the knitted fabric include a dappled pattern, dembigh, and half.

In the mesh knitted fabric of the invention, it is preferred that, for example, the mesh knitted fabric is knitted using the yarn composed of the conjugate fiber and the yarn used in the ground structure part, and then subjected to heat treatment by dyeing or the like, causing crimps in the conjugate fiber.

The temperature for the dyeing is preferably 100 to 140°C (more preferably 110 to 135°C), and, with respect to the time for the dyeing, the retention time at the highest temperature is preferably in the range of from 5 to 40 minutes. By dyeing the mesh knitted fabric under the above-mentioned conditions, the conjugate fiber causes crimps due to a difference in heat shrinkage between the polyester component and the polyamide component. In the conjugate fiber, by selecting the above-mentioned polymers as the polyester component and the polyamide component, a crimped structure is formed in which the polyamide component is positioned inside of the crimps.

It is preferred that the dyed mesh knitted fabric is subjected to dry heat final setting. The temperature for the dry heat final setting is preferably 120 to 200°C (more preferably 140 to 180°C), and the time for the dry heat final setting is preferably in the range of from 1 to 3 minutes. When the temperature for the dry heat final setting is lower than 120°C, there is a danger that wrinkles generated during dyeing are likely to remain, and further a finished product has poor dimensional stability. On the other hand, when the temperature for the dry heat final setting is higher than 200°C, it is likely that crimps caused in the conjugate fiber during dyeing are reduced, or that the fiber is hardened so that the resultant fabric has a hard hand feeling.

Further, the mesh knitted fabric of the invention preferably has been subjected to water absorption-imparting processing. By subjecting the mesh knitted fabric to water absorption-imparting processing, the knitted fabric is easily improved in the air permeability even with a small amount of sweat. The water absorption-imparting processing may be a general water absorption-imparting processing, and, as a preferred example, there can be mentioned a processing in which a water absorption imparting agent, such as polyethylene glycol diacrylate or a derivative thereof, or a polyethylene terephthalate-polyethylene glycol copolymer, is applied to the mesh knitted fabric in an amount of 0.25 to 0.50% by weight, based on the weight of the mesh knitted fabric. As examples of methods for water absorption-imparting processing, there can be mentioned a dye bath method in which a water absorption imparting agent is mixed into a dyeing liquid during dyeing, a method in which, before subjected to dry heat final setting, the fabric is dipped in a water absorption imparting liquid and squeezed by means of a mangle, and a method using an application method, such as a gravure coating method or a screen printing method.

Further, the weight ratio of the yarn composed of the conjugate fiber and the yarn used in the ground structure part (yarn composed of the conjugate fiber:yarn used in the ground structure part) is preferably in the range of from 5:95 to 30:70. The mesh knitted fabric of the invention is preferably comprised only of the conjugate fiber and the composite yarn (crimped fiber), but may further contain another fiber (for example, a non-crimped polyester multifilament).

The mesh knitted fabric of the invention preferably has a fiber areal weight of 250 g/m² or less (preferably 50 to 250 g/m², especially preferably 110 to 190 g/m²). When the fiber areal weight of the mesh knitted fabric is larger than 250 g/m², there is a danger that the mesh knitted fabric has such a large weight that the wear comfortability becomes poor, or that the movability (change in crimps) of the conjugate fiber in the mesh knitted fabric becomes poor. Further, the mesh knitted fabric preferably a knitted fabric density such that the number of courses is 20 to 100/2.54 cm and the number of wales is 20 to 80/2.54 cm. Particularly, when the knitted fabric density satisfies the above-mentioned ranges and the size of the mesh part (void) is in the above-mentioned range, the mesh knitted fabric is advantageously reversibly increased in the area of a mesh part when being wetted to such an extent that the increase of the area can be seen, enabling the self-regulating function of the fabric to be visually recognized.

In the thus obtained mesh knitted fabric, as diagrammatically shown in FIG. 3, the yarn composed of the conjugate fiber is used in the connecting part for connecting the ground structure parts adjacent to each other, and therefore, when the mesh knitted fabric is wetted, the conjugate fiber stretches in the widthwise direction, and accordingly, the mesh part also expands in the widthwise direction. As a result, the mesh knitted fabric is reversibly improved in air permeability, and further the expansion of the mesh part enables the effect of improvement to be visually recognized.

The area of the mesh part may expand to such an extent that expansion of the area can be visually recognized, but it is preferred that the area of the mesh of the mesh knitted fabric upon being wetted is 1.1 times or more (more preferably 1.1 to 20 times, especially preferably 2 to 10 times) the area of the mesh before wetted.

Further, the air permeability change ratio represented by the formula below is preferably 5% or more (more preferably 50 to 500%). An air permeability of the fabric is a value (c.f.m.) as measured in accordance with JIS L1096-2010, 8.26.1, A method (Frajour type method) (wherein the pressure for measurement is changed from 125 Pa described in JIS to 20 Pa). Air permeability change ratio (%) = (((Air permeability of the wetted fabric) - (Air permeability of the dried fabric))/(Air permeability of the dried fabric)) × 100

The dried fabric means a fabric in the state obtained after allowing a fabric sample to stand in an environment at a temperature of 20°C and at a humidity of 65% RH for 24 hours. On the other hand, the wetted fabric means a fabric in the state obtained after causing a fabric to uniformly contain water in an amount of 50% by weight, based on the weight of the fabric, and then allowing the resultant fabric to stand for one minute, and air permeability values (n = 5) of each of the dried and wetted fabric samples are measured, and their respective averages are determined.

When the air permeability change ratio of the fabric is smaller than 5%, there is a disadvantage in that a problem of uncomfortable sweaty feeling is likely to occur upon sweating. It is preferred that, after the fabric is washed once in accordance with JIS L0217-1995, 103 method, the air permeability change ratio of the fabric is preferably 10% or more (more preferably 30 to 500%, especially preferably 50 to 100%).

Further, the dimensional change ratio of the cloth, in terms of an absolute value, is preferably 10% or less in the lengthwise direction and/or 15% or less in the widthwise direction. Particularly, the dimensional change ratio is preferably -3 to +3% (more preferably -2 to +2%) both in the lengthwise direction and in the widthwise direction. The dimensional change ratio of the cloth is represented by the following formula. Dimensional change ratio of the cloth (%) = (((Dimension of the wetted cloth) - (Dimension of the dried cloth))/(Dimension of the dried cloth)) × 100

The dried cloth means a cloth in the state obtained after allowing a cloth sample having a dimension (length: 20 cm × width: 2.5 cm = 50 cm²) to stand in an environment at a temperature of 20°C and at a humidity of 65% RH for 24 hours. Five samples are prepared for the measurement of dimension for each of the length and width. On the other hand, the wetted cloth means a cloth in the state obtained after immersing a cloth sample in water at a temperature of 20°C for 10 minutes, and then immediately hanging the resultant cloth in the long direction for 5 minutes, and dimension values (the number of samples = 5) of each of the dried and wetted cloth samples are measured, and their respective averages are determined.

When the dimensional change ratio of the cloth is larger than the above-mentioned range, there is a disadvantage in that a fiber product obtained from the resultant mesh knitted fabric is poor in wear comfortability or appearance. It is preferred that, after the cloth is washed once in accordance with JIS L0217-1995, 103 method, the dimensional change ratio of the cloth is 10% or less in the lengthwise direction and/or 15% or less in the widthwise direction.

With respect to the mesh knitted fabric of the invention, in addition to the above-mentioned processing, processing for imparting a function, such as raising according to a general method, ultraviolet light screening, or processing using an anti-fungus agent, a deodorant, an insectifuge, a phosphorescent material, a retroreflective material, a negative ion generator, a water repellent, or the like, may be additionally applied to the mesh knitted fabric.

Further, in the invention, there is provided a fiber product which is obtained using the above-described mesh knitted fabric, wherein the fiber product is selected from the group consisting of clothes, a backing fabric, a core fabric, socks, a stomach band, a hat, gloves, nightclothes, a casing material for futon (thick bedquilt), a cover for futon, and a car seat skin material. The fiber product uses the above-described cloth, and therefore is reversibly increased in the area of a mesh part when being wetted, enabling the self-regulating function of the fiber product to be visually recognized.

### Examples

Hereinbelow, the present invention will be described in more detail with reference to the following Examples, which should not be construed as limiting the scope of the present invention. In the following Examples, physical properties were measured in accordance with the methods described below.

### (1) Intrinsic viscosity of polyester

An intrinsic viscosity of polyester is measured at a temperature of 35°C using orthochlorophenol as a solvent.

### (2) Intrinsic viscosity of polyamide

An intrinsic viscosity of polyamide is measured at a temperature of 30°C using m-cresol as a solvent.

### (3) Washing and drying

Washing is conducted once in accordance with JIS L0217-1995, 103 method. Further, drying is conducted in accordance with JIS L1096-2010, 8.24.1, A1 method-2.3 tumbler.

### (4) Air permeability change ratio

An air permeability of the fabric is a value (c.f.m.) as measured in accordance with JIS L1096-2010, 8.26.1, A method (Frajour type method) (wherein the pressure for measurement is changed from 125 Pa described in JIS to 20 Pa). The dried fabric (DRY) means a fabric in the state obtained after allowing a fabric sample to stand in an environment at a temperature of 20°C and at a humidity of 65% RH for 24 hours. On the other hand, the wetted fabric (WET) means a fabric in the state obtained after causing a fabric to uniformly contain water in an amount of 50% by weight, based on the weight of the fabric, and then allowing the resultant fabric to stand for one minute, and air permeability values (the number of samples = 5) of each of the dried and wetted fabric samples are measured, and their respective averages are determined. Then, an air permeability change ratio is determined from the following formula. Air permeability change ratio (%) = (((Air permeability of the wetted fabric)) - (Air permeability of the dried fabric))/(Air permeability of the dried fabric)) × 100

### (5) Dimensional change ratio

A dimension for length (width) of the dried cloth and a dimension for length (width) of the wetted cloth are measured.

The dried cloth means a cloth in the state obtained after allowing a cloth sample having a dimension (length: 20 cm × width: 2.5 cm = 50 cm²) to stand in an environment at a temperature of 20°C and at a humidity of 65% RH for 24 hours. Five samples are prepared for the measurement of dimension for each of the length and width. On the other hand, the wetted cloth means a cloth in the state obtained after immersing a cloth sample in water at a temperature of 20°C for 10 minutes, and then immediately hanging the resultant cloth in the long direction for 5 minutes, and dimension values (the number of samples = 5) of each of the dried and wetted cloth samples are measured, and their respective averages are determined. Then, a dimensional change ratio of the cloth is determined from the following formula. Dimensional change ratio of the cloth (%) = (((Dimension of the wetted cloth) - (Dimension of the dried cloth))/(Dimension of the dried cloth)) × 100

### (6) Dimensional change ratio between the washed cloth and the cloth before washed

A dimension for length (width) of the cloth before washed and a dimension for length (width) of the washed cloth are measured. Then, a dimensional change ratio of the cloth is determined from the following formula. Dimensional change ratio (%) = ((Dimension of the cloth before washed) - (Dimension of the washed cloth)) / (Dimension of the cloth before washed) × 100

### (7) Fiber areal weight

A fiber areal weight is measured in accordance with JIS L1018-1998 6.4.

### (8) Expansion of the mesh part

A fabric sample was allowed to stand in an environment at a temperature of 20°C and at a humidity of 65% RH for 24 hours, and then an area of the mesh part of the resultant fabric in this state was measured using an optical microscope. Then, the fabric was caused to uniformly contain water in an amount of 50% by weight, based on the weight of the fabric, and then allowed to stand for one minute, and an area of the mesh of the resultant fabric in this state was measured using an optical microscope, determining which times the area of the mesh part of the wetted fabric is, as compared to the (original) area of the mesh part before wetted. The number of samples was 3, and an average of the measured values was determined. Further, a sample such that expansion of the mesh upon being wetted could be visually recognized was rated "O", and a sample such that expansion of the mesh upon being wetted could not be visually recognized was rated "Δ".

### [Example 1]

As yarn type 1 (for ground structure), a semi-dull polyester multifilament (44 dtex/48 filaments) was prepared.

Separately, nylon 6 having an intrinsic viscosity [η] of 1.3 and modified polyethylene terephthalate having an intrinsic viscosity [η] of 0.39 and having copolymerized therewith sodium 5-sulfoisophthalate in an amount of 2.6 mol% were melted respectively at 270°C and 290°C, and individually extruded using a composite spinning nozzle similar to FIG. 1 of JP2000-144518A at an extrusion rate of 12.7 g/minute to form a conjugate fiber having a single-yarn transverse cross-sectional shape in a side-by-side form. The conjugate fiber was solidified by cooling and an oil agent was applied thereto and then, the resultant yarn was preheated using preheating rollers at a rate of 1,000 m/minute and at a temperature of 60°C, and then subjected to drawing heat treatment between the preheating rollers and heating rollers heated to a temperature of 150°C at a rate of 3,050 m/minute, and wound up to obtain a yarn composed of a conjugate fiber (total fineness: 84 dtex/24 filaments) as yarn type 2 (for connecting part).

Subsequently, using a 28-gauge warp knitting machine, as shown in FIG. 1, raveling was made according to the followings: yarn type 1: 13 in, 1 out (10/12); yarn type 1: 13 in, 1 out (12/10); yarn type 2: 11 out, 2 in, 1 out (10/45: 9 repeats; 10/12: 2 repeats), and a warp-knitted fabric (mesh knitted fabric) having a mesh structure (in which one mesh part has a size of 4 courses and 1 wale) was knitted.

Then, the warp-knitted fabric was dyed at a temperature of 130°C for a retention time of 15 minutes so that the latent crimping performance of the conjugate fiber was actualized. In this instance, a water absorption imparting agent (polyethylene terephthalate-polyethylene glycol copolymer) was added to the dyeing liquid in an amount of 2 ml/l, and the knitted fabric was treated in the same bath for the dyeing, applying the water absorption imparting agent to the knitted fabric. Then, the resultant warp-knitted fabric was subjected to dry heat final setting at a temperature of 160°C for a period of time of one minute.

The obtained knitted fabric had excellent air permeability changing function upon being wetted and excellent dimensional stability. Further, when the knitted fabric was wetted, expansion of the mesh part could be visually recognized (the area of the mesh part of the mesh knitted fabric upon being wetted was 4.12 times the area of the mesh part before wetted). The results of the evaluation are shown in Table 1.

Further, clothes were obtained using the knitted fabric and worn. As a result, it was found that the clothes had excellent air permeability changing function upon being wetted and excellent dimensional stability.

### [Example 2]

Polyethylene terephthalate (matting agent content: 0.3% by weight) was melt spun from a general spinning apparatus at 280°C, and taken up at a rate of 2,800 m/minute and wound without being drawn, obtaining a semi-drawn polyester yarn (total fineness: 56 dtex/24 filaments; single fiber cross-sectional shape: circular cross-section). Then, the obtained polyester yarn was subjected to co-drawing false-twist crimping under conditions such that the draw ratio was 1.6 times, the number of false-twists was 2,500 T/m (in the S direction), the heater temperature was 180°C, and the yarn speed was 350 m/minute.

Further, the polyester yarn was subjected to co-drawing false-twist crimping under conditions such that the draw ratio was 1.6 times, the number of false-twists was 2,500 T/m (in the Z direction), the heater temperature was 180°C, and the yarn speed was 350 m/minute. Then, the false-twisted crimped yarn having a torque in the S direction and the false-twisted crimped yarn having a torque in the Z direction were doubled and subjected to air interlacing treatment, obtaining a composite yarn (total fineness: 66 dtex/48 filaments) as yarn type 1.

Then, yarn type 2 which is the same as that in Example 1 was obtained, and a warp-knitted fabric (mesh knitted fabric) having a mesh structure (in which one mesh part has a size of 4 courses and 1 wale) was knitted in substantially the same manner as in Example 1 except that the knitted fabric density was changed as shown in Table 1.

The obtained knitted fabric had excellent air permeability changing function upon being wetted and excellent dimensional stability. Further, when the knitted fabric was wetted, expansion of the mesh part could be visually recognized (the area of the mesh part of the mesh knitted fabric upon being wetted was 2.42 times the area of the mesh part before wetted). The results of the evaluation are shown in Table 1.

Further, clothes were obtained using the knitted fabric and worn. As a result, it was found that the clothes had excellent air permeability changing function upon being wetted and excellent dimensional stability.

### [Comparative Example 1]

As yarn type 1, a semi-dull polyester multifilament (110 dtex/144 filaments) was prepared. Separately, yarn type 2 which is the same as that in Example 1 was obtained.

Subsequently, using a 28-gauge circular knitting machine, the yarn type 1 and yarn type 2 were paralleled, and a circular knitted fabric was knitted according to a smooth structure (having no mesh part) shown in FIG. 2.

Then, the circular knitted fabric was dyed at a temperature of 130°C for a retention time of 15 minutes so that the latent crimping performance of the conjugate fiber was actualized. In this instance, a water absorption imparting agent (polyethylene terephthalate-polyethylene glycol copolymer) was added to the dyeing liquid in an amount of 2 ml/l, and the knitted fabric was treated in the same bath for the dyeing, applying the water absorption imparting agent to the knitted fabric. Then, the resultant circular knitted fabric was subjected to dry heat final setting at a temperature of 160°C for a period of time of one minute.

The obtained circular knitted fabric had excellent air permeability changing function upon being wetted and excellent dimensional stability, but, when the knitted fabric was wetted, the self-regulating function could not be visually recognized. The results of the evaluation are shown in Table 1.

**[Table 1]**

| | | Example 1 | Example 2 | Comparative Example 1 |
|---|---|---|---|---|
| Knitting design | Gauge | 28G | 28G | 28G |
| | Structure | Warp knitted Mesh (FIG. 1) | Warp knitted Mesh (FIG. 1) | Circular knitted Smooth (FIG. 2) |
| Yarn type | Yarn type 1 | SD 44T48 | Composite yarn SD 66T48 | SD 110T144 |
| | Yarn type 2 | SDD 84T24 | SDD 84T24 | SDD 84T24 |
| Knitted fabric | Knitted fabric density | 58/49 | 52/44 | 52/45 |
| | Fiber areal weight (g/m²) | 137 | 154 | 140 |
| Before washed | Air permeability (DRY) | 109 | 135 | 60 |
| | Air permeability (WET) | 173 | 189 | 68.4 |
| | Air permeability change ratio (%) | 58.7 | 40 | 14 |
| After washed | Air permeability (DRY) | 92 | 114 | 50 |
| | Air permeability (WET) | 163 | 174 | 66 |
| | Air permeability change ratio (%) | 77.9 | 52.6 | 32 |
| Dimensional change ratio (%) upon being wetted (Lengthwise × Widthwise) | Before washed | 1.3 × 9.9 | 0.6 × 9.5 | 3.5 × 1.5 |
| | After washed | 1.7 × 11.5 | 1.0 × 6.1 | 4.5 × 2.0 |
| Dimensional change ratio (%) between before and after washed (Lengthwise × Widthwise) | | 0.3 × 1.4 | 0.1 × 1.3 | 3.2 × 1.5 |
| Weight ratio (Yarn type 1:Yarn type 2) | | 19:81 | 14:86 | 27:73 |
| Appearance change can be visually recognized or not | | ○ | ○ | Δ |

### Industrial Applicability

In the present invention, there are provided a mesh knitted fabric which is reversibly increased in the area of a mesh part when being wetted, enabling the self-regulating function of the fabric to be visually recognized, and a fiber product, and such a fabric and fiber product are of extremely great commercial significance.

### Reference Signs List

- 1:: Mesh part
- 2:: Connecting part
- 3:: Ground structure part

## Claims

1. A mesh knitted fabric having a mesh part, wherein the mesh knitted fabric comprises a yarn composed of a conjugate fiber having a polyester component and a polyamide component bonded in a side-by-side form, wherein the area of the mesh part of the mesh knitted fabric upon being wetted is increased, as compared to the area of the mesh part before wetted.

2. The mesh knitted fabric according to claim 1, wherein the size of the one mesh part is in the range of from 2 to 12 courses.

3. The mesh knitted fabric according to claim 1, which further comprises a composite yarn containing a false-twisted crimped yarn having a torque in the S direction and a false-twisted crimped yarn having a torque in the Z direction.

4. The mesh knitted fabric according to claim 1, which has a warp-knitted fabric structure.

5. The mesh knitted fabric according to claim 1, which has a knitted fabric density wherein the number of courses is 20 to 100/2.54 cm and the number of wales is 20 to 80/2.54 cm.

6. The mesh knitted fabric according to claim 1, which contains a water absorption imparting agent.

7. The mesh knitted fabric according to claim 1, which has a fiber areal weight in the range of from 50 to 250 g/m².

8. The mesh knitted fabric according to claim 1, which has an air permeability change ratio of 5% or more when being wetted.

9. The mesh knitted fabric according to any one of claims 1 to 8, which has a dimensional change ratio of 10% or less in the lengthwise direction and a dimensional change ratio of 15% or less in the widthwise direction when being wetted.

10. A fiber product which is obtained using the mesh knitted fabric according to any one of claims 1 to 9, wherein the fiber product is selected from the group consisting of clothes, a backing fabric, a core fabric, socks, a stomach band, a hat, gloves, nightclothes, a casing material for futon (thick bedquilt), a cover for futon, and a car seat skin material.
